

## UNITED STATES PATENT OFFICE

1,945,737

## HEAT TREATMENT OF ALUMINUM-MAGNESIUM ALLOYS

Edgar H. Dix, Jr., Oakmont, Pa., and Louis W. Kempf, Cleveland, Ohio, assignors to Aluminum Company of America, Pittsburgh, Pa., a corporation of Pennsylvania

No Drawing. Application December 23, 1930  
Serial No. 504,278

6 Claims. (Cl. 148—21.1)

This invention relates to aluminum base alloys containing substantial amounts of magnesium, and one of its objects is to improve the physical properties of this class of alloys by suitable heat treatments. Another object is to regulate or alter by heat treatment certain of the physical properties of articles made from these alloys to produce various commercially useful conditions in the internal structure of the articles.

The recent successful developments in the production of aluminum base alloys containing substantial amounts of magnesium have now made possible the production of clean sound castings of aluminum base alloys with magnesium within the range where the greatest difficulty was formerly encountered, namely, from about 5 per cent to about 20 per cent of magnesium.

The low specific gravity of magnesium makes it a very desirable constituent in aluminum alloys but because of the difficulties heretofore encountered in making clean and sound castings of such alloys containing more than about 5 per cent magnesium, alloys of this type have not been used to any extent except in rare instances where the ordinary standards of tensile strength, ductility and soundness were made subservient to some other property usually not seriously considered in appraising the usefulness of an alloy.

Simultaneously with the development of casting methods as noted above, we have been investigating the possibility of improvement or alteration of the properties and internal structure of these alloys by causing the soluble constituent or constituents of the alloy to go into solid solution, and the methods of heat-treatment by which such properties and qualities are produced are embraced within the subject matter of the present application. We have found that the herein described alloys are susceptible to improvement by heat treatment both in the "as-cast" and in the "worked" condition, the working being effected by any of the known methods, such as rolling, forging, extrusion, etc.

In practicing one of the steps of our invention we take an aluminum base alloy casting containing from about 5 per cent to 20 per cent magnesium and perhaps smaller quantities of other alloying elements and heat it for a period of time at a temperature such as hereinafter discussed.

We have found it necessary to keep the casting at heat at least 5 hours to produce advantageous effects and for the best results a considerable increase in time is desirable. As a standard heat treating time we use 20 hours although times even longer than this have been found of advantage in the case of the higher amounts of magnesium. Articles which have been rolled, forged, extruded, or otherwise subjected to working processes will respond to heat treatment more rapidly than castings although they may, with good effect, be given the same treatment as that outlined above.

As indicating the beneficial effect of extended time at heat, we give below in Table A typical results with sand cast tensile specimens containing 14 per cent magnesium and heat treated at 445° C. for the times stated in the table. The specimens were cooled by air blast:

Table A

| Hours at 445° C. | Tensile strength<br>lbs. per<br>sq. in. | Elongation<br>in 2" |
|------------------|-----------------------------------------|---------------------|
| 24.....          | 41,550                                  | 5.2                 |
| 72.....          | 48,760                                  | 12.4                |

With lower amounts of magnesium the heat treating temperature may be somewhat reduced and the time somewhat shortened. The following Table B shows the effect of heat treating sand cast tensile specimens of 10 per cent magnesium, balance aluminum, at 427° C., for the times indicated.

Table B

| Hours at 427° C. | Tensile strength<br>lbs. per<br>sq. in. | Elongation<br>in 2" |
|------------------|-----------------------------------------|---------------------|
| 2.....           | 36,230                                  | 7.3                 |
| 24.....          | 39,207                                  | 10.0                |
| 72.....          | 41,500                                  | 11.9                |

As described in a copending application of L. W. Kempf, Serial No. 454,523, a material improvement in properties accompanies the use of high purity ingredients for compounding the

alloys, whereby iron, silicon, and other impurities are held to a relatively low figure. In such alloys the beneficial effects of extended time at heat are especially evident, as illustrated in Table 5 C below. The tensile specimens were cast in sand from an alloy containing 10 per cent magnesium, were heat treated at 425° C. for the times indicated in the table, and were tested three days after quenching. The alloy was made 10 using aluminum ingot containing not more than 0.3 per cent impurities.

Table C

| 15 | Hours at 425° C. | Tensile strength lbs. per sq. in. | Elongation in 2" |
|----|------------------|-----------------------------------|------------------|
| 1  |                  | 44,600                            | 13.5             |
| 5  |                  | 46,700                            | 16.0             |
| 20 |                  | 50,400                            | 19.5             |

With extended time a marked increase in both tensile strength and elongation is noted, and for this reason when heat treating quantities of 25 miscellaneous castings we prefer to use at least 20 hours, even extending this time if optimum results are needed.

We prefer to restrict our heat treating range to lower than 451° C., as we have observed that 30 at this temperature the magnesium constituent which has not gone into solution forms a low melting point aggregate with the aluminum matrix. Temperatures in the neighborhood of 330° to 425° C. have been found to be of fairly 35 general usefulness, and for the best results articles should be heated as high as convenient without too closely approaching 451° C. Higher temperatures have the effect of shortening the time in which identical results are obtained, and 40 with lower temperature the time at heat is correspondingly lengthened. Temperatures as low as 250° C. effect an advantageous improvement, especially with alloys of lower magnesium contents, such as those in the neighborhood of 5 45 per cent. As the amount of magnesium is increased we find it advantageous to raise the temperature, and in ordinary commercial practice we usually employ a standard temperature of 425° C.

50 With magnesium contents higher than about 10 per cent we have found that if heated articles are quenched in water cracks may form which will render the articles useless or cause considerable decrease in strength and ductility. We 55 have also found that if the specimens be cooled more slowly, as in air, the results are highly satisfactory. Articles may even be slowly cooled in the furnace over a period of several hours to about 300° C. and then cooled in air without appreciable diminution in properties. This characteristic of the alloy is especially useful in the case of articles which by reason of intricacy of 60 design or variation of section show a tendency to crack if rapidly quenched, and in this respect 65 our method differs notably from that practiced in the case of other commercial aluminum alloys.

We have found that lesser amounts of other 70 alloying constituents may be included without rendering the alloy insensitive to improvement by heat treatment and, as a matter of fact, sometimes enhancing the improvement obtained. As an instance of the effect of adding 0.5 per cent of zinc to an aluminum base alloy containing 10 per cent magnesium, we have tested specimens 75 of this composition both in the "as-cast" condi-

tion and after a heat treatment of 20 hours at 425° C. with the results shown in the following Table D:

Table D

| Condition         | Tensile strength lbs. per sq. in. | Elongation in 2" | 80 |
|-------------------|-----------------------------------|------------------|----|
| As-cast.....      | 21,420                            | 0.5              | 85 |
| Heat-treated..... | 48,320                            | 17.0             |    |

We have found that the usefulness of these heat treating processes is not restricted to "as-cast" articles but that the processes may also be directed towards the alteration or improvement of the properties and internal structure of wrought articles fabricated by such methods as rolling, forging, extrusion, pressing, etc. 90

We have also found that the alloys within the scope of this invention are susceptible to increase the tensile strength and hardness by being subjected to heating for extended periods of time at lower temperatures. Table E, immediately 100 below, indicates the effect on tensile specimens of aging at 154° C. after a high temperature treatment. The tensile specimens were cut from 14 gage sheet made from an aluminum base alloy containing 10 per cent of magnesium. 95

Table E

| Condition              | Tensile strength lbs. per sq. in. | Elongation in 2" | Sclerometer hardness | 105 |
|------------------------|-----------------------------------|------------------|----------------------|-----|
| As-quenched.....       | 51,370                            | 30.5             | 17.0                 | 110 |
| 24 hrs. at 154° C..... | 53,620                            | 30.5             | 19.0                 |     |
| 70 hrs. at 154° C..... | 58,400                            | 22.7             | 22.5                 |     |

In aluminum base alloys containing magnesium in amounts ranging from about 5 per cent to about 20 per cent the heat treating processes described in this specification may be utilized even though there be present one or more other alloying constituents in lesser amounts. Certain 115 alloying elements in addition to magnesium, as for example manganese, chromium, and nickel, are even found to be distinctly helpful in imparting additional improvement effects to the articles heat treated by the methods herein disclosed. It should also be understood that the aluminum ingot used in compounding these alloys 120 may contain an appreciable amount of impurities such as iron, silicon, copper and lesser quantities of other elements and that some of these 125 may combine with a relatively small amount of the magnesium or may form compounds with each other, and may be caused to undergo structural variations by our heat treating process, but although we recognize the presence of these elements 130 we do not regard them as essential to the success of the heat treating processes we have devised, and we may, in certain cases, even desire to eliminate as far as possible these impurities as being detrimental to the best properties 135 in the alloy. As an aid in outlining the limits of the invention, we postulate an alloy of an aluminum base with magnesium varying between the limits 5 and 20 per cent and have devised 140 heat treating methods applicable to this class of alloys whether or not other alloying elements are present and whether or not these alloying elements are present as impurities or as intentional additions with the end in view of improving 145 the alloys so heat-treated. 150

## We claim—

1. The method of treating an aluminum base alloy containing from about 5 to 20 per cent magnesium to improve the physical properties thereof, comprising heating the alloy for about 5 to 20 hours at a temperature from about 250° to 450° C., and cooling the alloy rapidly enough to preserve the benefits of the heating.

2. The method of treating an aluminum base alloy containing from about 10 per cent to 20 per cent magnesium to improve the physical properties thereof, which comprises heating the alloy between about 380° C. and about 450° C. for about 5 to 20 hours, and cooling the alloy rapidly enough to preserve the benefits of the heating.

3. The method of treating an aluminum base alloy containing from about 5 to 15 per cent magnesium and not more than 2 per cent of another metallic element of the class composed of manganese, chromium, nickel and zinc, comprising heating the alloy at a temperature from about 250° C. to about 450° C. for about 5 to 20 hours, and cooling the alloy from the temperature of the heating.

4. The method of treating an aluminum base alloy containing from about 5 per cent to about 20 per cent magnesium, which comprises heating the alloy for more than 5 hours but not more

than 20 hours at from about 250° C. to about 450° C., cooling the alloy rapidly enough to retain the benefits of the heat treatment, and thereafter re-heating the alloy at a temperature less than 200° C. for a period of time sufficient to increase the strength and hardness of the alloy.

5. The method of treating a casting made of an aluminum base alloy containing from about 5 to 20 per cent magnesium, which comprises heating the casting for more than about 5 but not more than about 20 hours, at from about 250° C. to about 450° C., cooling the casting rapidly enough to retain the benefits of the heat treatment but slowly enough to avoid cracking of the casting, and thereafter re-heating the alloy at a temperature from about 150° C. to 200° C. to increase the strength and hardness of the casting.

6. The method of treating a casting made of an aluminum base alloy containing from about 5 to 20 per cent magnesium comprising heating the casting for more than about 5 hours but not more than about 20 hours at a temperature of from 425° C. to 450° C., cooling the casting slowly to about 300° C., and then cooling the casting in air to room temperature.

EDGAR H. DIX, JR.  
LOUIS W. KEMPF.

30

105

35

110

40

115

45

120

50

125

55

130

60

135

65

140

70

145

75

150